

## UNITED STATES PATENT OFFICE

1,973,422

## HARD METAL COMPOSITION

Elmer B. Welch, McKeesport, Pa., assignor to  
Firth-Sterling Steel Company, McKeesport, Pa.,  
a corporation of Pennsylvania

No Drawing. Application April 28, 1933,  
Serial No. 668,386

6 Claims. (Cl. 75—1)

This invention relates to hard metal compositions useful in the production of cutting tools, wire drawing dies, and the like. It relates more particularly to such a composition containing 5 titanium carbide, tungsten and aluminum.

The metallic tungsten, taken in conjunction with the aluminum, preferably constitutes at least 50% of the composition. The composition of the present invention differs from certain hard 10 metal compositions known heretofore and which contained a relatively large proportion of a hard metal carbide such as tungsten carbide and a relatively small proportion of an auxiliary metal such as cobalt, nickel or iron. In the composition 15 of the present invention, the titanium carbide preferably constitutes only a minor proportion of the total composition, the metallic constituents, namely, the tungsten and aluminum, preferably constituting at least 50% of the composition. 20

The titanium carbide may vary between 15 and 60%, but preferably between 20 and 50%. In a preferred composition, it constitutes about 32%. The tungsten may vary between 25 and 82%, but 25 preferably is between 40 and 74%. In a preferred composition, it constitutes about 60%. The aluminum may vary between 3 and 15%, preferably between 6 and 10%, and in a preferred composition it constitutes about 8% of the total composition. 30

The composition may be made by sintering, welding, fusing or melting the constituents. If a sintered composition is to be produced, titanium carbide, metallic tungsten, and aluminum, all in 35 finely powdered form, are mixed together as by rolling them in a rolling barrel and are thereafter sintered at a temperature of about 3000° F. The mixed powders may be first compacted and then sintered, either with or without a preliminary sintering at a lower temperature, or the 40 mixed powders may be compacted and sintered simultaneously in accordance with the hot press method. Where the mixture is first compacted and then sintered, it is preferred to carry out the sintering step in a hydrogen or other reducing atmosphere. 45

It has been found that cobalt, nickel or iron, which are the auxiliary metals most commonly used in producing hard cemented carbide materials, have an embrittling effect if present in my 50 composition in amounts of 4 or 5% or more, or to some extent even when present in about 2% of the composition. It is preferred, therefore, in my composition not to use these auxiliary metals, 55 or if they are present, to keep them below about

4 or 5%, and preferably below 2% of the composition.

My composition, wherein the titanium carbide preferably constitutes only a minor proportion of the composition, is easier to compress than compositions containing a relatively large amount of a hard metal carbide and a relatively small amount of auxiliary metal. The ease of compressing my composition facilitates its manufacture and the composition has less abrasive effect 60 on the dies in which it is compressed than other compositions having a higher proportion of hard metal carbide. My preferred composition has a Rockwell C hardness of about 78, which is approximately equal to the hardness of a composition containing about 94% of tungsten carbide and 6% of cobalt. My composition, containing a relatively small amount of titanium carbide, is more economical to produce than other compositions containing larger amounts of the carbide, and yet has proved to be an excellent steel 75 cutting material.

The aluminum lowers the sintering temperature and, in addition, imparts hardness as well as age hardening properties to the composition. 80 A portion of the aluminum may be replaced by magnesium or beryllium in order to give increased hardness to the composition.

I have described the present preferred embodiment of my invention and have described one 85 method of making the composition. It is to be understood, however, that the invention may be otherwise embodied or practiced within the scope of the following claims.

I claim:

1. A hard metal composition consisting of about 15 to 60% of titanium carbide, about 25 to 82% of tungsten, and about 3 to 15% of aluminum.

2. A hard metal composition consisting of about 20 to 50% of titanium carbide, about 40 to 74% of tungsten, and about 3 to 15% of aluminum. 95

3. A hard metal composition consisting of about 15 to 60% of titanium carbide, about 25 to 82% of tungsten, and about 6 to 10% of aluminum.

4. A hard metal composition containing about 100 32% of titanium carbide, about 60% of tungsten, and about 3 to 15% of aluminum.

5. A sintered hard metal composition consisting of about 15 to 60% of titanium carbide, about 25 to 82% of tungsten, and about 3 to 15% of aluminum. 105

6. A sintered hard metal composition consisting of about 20 to 50% of titanium carbide, about 40 to 74% of tungsten, and about 3 to 15% aluminum.